

## UNITED STATES PATENT OFFICE.

WILLIAM WARWICK STENNING AND WALTER HENRY BEASLEY, OF LONDON, ENGLAND, ASSIGNORS TO MINERALS SEPARATION NORTH AMERICAN CORPORATION, OF NEW YORK, N. Y.

## TREATMENT OF FINELY-DIVIDED COAL.

No Drawing.

Application filed February 15, 1922. Serial No. 598,210.

To all whom it may concern:

Be it known that we, WILLIAM WARWICK STENNING and WALTER HENRY BEASLEY, both subjects of the King of England, residing at London, in England, have invented certain new and useful Improvements in the Treatment of Finely-Divided Coal, of which the following is a specification.

10 This invention consists in improvements in or relating to the production of coal briquettes. One of the objects of this invention is to facilitate the production of coal briquettes from flotation concentrates, although the invention is also applicable to the production of coal briquettes from other coal concentrates or from finely divided coal.

In British Patent No. 155875 a process is described in which the coal concentrate or finely divided coal suspended in water is subjected to agitation (preferably with aeration) with a liquefied binding medium, such as melted pitch, with or without tar, resin and the like, whereby the coal particles become coated with the binding medium and flocculated so as to be readily separable from the water. We make no claim to anything described or claimed in that patent.

Investigations have been carried out on the treatment of an aqueous suspension of finely divided coal or coal concentrates with the addition of a binding medium, such as pitch, to ascertain whether agglomeration can be improved, particularly by eliminating air and also by heating the suspension to facilitate the distribution of the binding medium, such as pitch, over the surfaces of the coal particles, and the results of these investigations have been most striking.

According to this invention a step in the process of producing briquettes from finely divided coal or from coal concentrates, is characterized by the fact that the finely divided coal suspended in water and mixed with a binding medium (such as finely divided pitch, with or without an added agent such as naphthalene or tar, which causes the pitch, when softened, to spread over the surfaces of the coal particles) is subjected to such conditions, as, for example to heat, that the binder will flow and will coat the coal particles and to such agitation as will elim-

inate air to ensure the agglomeration of the coal particles before pressing the agglomerate into briquettes.

In certain cases the agents employed for agglomeration may be strong binders which lead to the eventual production of strong briquettes, but as one main object in view is the elimination of water from wet concentrate, it may be sufficient in some cases to employ other agglomerating agents which are not generally recognized as binders. In these cases also, to facilitate handling, the treated coal may be pressed into blocks which although relatively soft are sufficiently coherent and are herein referred to as briquettes.

Particularly successful results have been obtained by the use of a rolling form of agitation without aeration in which the solid particles or solids are caused to roll upon the interior surface of the agitating vessel with the result that they tend to adhere together and form agglomerates. The rolling form of agitation which is common in the manufacture of certain sweets, can readily be secured in a horizontal rotating barrel or the equivalent.

This invention includes a process of making coal briquettes from finely divided coal or from coal concentrates, in which the finely divided coal, suspended in water, is mixed with a binding medium of the kind described (preferably by agitation accompanied by aeration) to ensure the dissemination of the binding medium, after which the suspension is heated substantially to boiling point and subjected to a rolling form of agitation to ensure the agglomeration of the coal particles, which are then formed into briquettes. Preferably, according to this invention, the agglomerate is introduced into the briquetting press while it is still hot, so that the binding medium is still soft. Further, according to this invention, the agglomerate after being submitted to the rolling form of agitation or such other agitation as will eliminate air, is introduced into the briquetting press with no further preparation than the rough draining of the now readily separable water.

The finely divided coal under treatment

is preferably suspended in the minimum of water necessary to form a mobile pulp which can be readily agitated or stirred. For example, the material treated may be flotation coal concentrates which carry about their own weight of water.

According to this invention the rolling agitation may be effected in a drum rotating on a substantially horizontal axis, with or without rods therein to knead or roll the agglomerating coal particles.

The invention will best be understood by the description of actual tests.

Some Powell Duffryn coal crushed to pass  $\frac{1}{16}$ th inch aperture (i. e. to 5 mesh I. M. M.), was subjected to flotation treatment in a minerals separation circulating machine, (such as is shown in Figure 3 of Lyster Patent No. 1,203,772 of October 31, 1916) with the addition of the equivalent of  $\frac{2}{3}$ rd lb. of cresol per ton of coal and  $\frac{1}{3}$ rd lb. of kerosene oil per ton of coal. The resulting float contained about equal parts of coal and water. This was introduced into a mineral separation agitation vessel, where the 1:1 pulp was quite mobile, and was agitated with aeration while there was added a quantity of pitch ground to minus 100 mesh I. M. M., amounting to 5% on the dry coal, also a quantity of ordinary gas tar, amounting to 2% on the dry coal. The whole pulp was then introduced into a horizontal cylinder with annular end plates (similar to a rotary kiln). Two long cylindrical rods were put in the bottom of the cylinder, and the cylinder was rotated on its own axis over a burner, so as to heat the pulp. The agitation was such as to avoid aeration—on the contrary any air entangled among the particles appeared to be eliminated. At a temperature of about 80° C. the agglomeration of the coated particles was very noticeable. The whole pulp was heated up to boiling point, the rolling agitation continuing. After this operation a sample of the pulp was placed on a 60 mesh screen, and it was noticed that the agglomerated coal remained on the screen, and the water which passed through the screen was perfectly clear; indeed, the agglomeration was such that the water very readily drained away from the agglomerate, whereas before this treatment of heating and agitation for elimination of air, the water in this test was not clear and could not be readily separated from the coal and binding media.

In a further test on this coal the same results were obtained when adding the pitch in a molten condition during the preliminary agitation with aeration instead of as a finely ground powder.

The agglomerated material, while still hot, was introduced in suitable quantities into a briquetting press, and satisfactory

briquettes were very readily made therefrom.

In the example given above the 2% of gas tar may conveniently be replaced by 1% of naphthalene, or a mixture of tar and naphthalene. The proportions of these ingredients may be varied; good results have been obtained using 0.05% of naphthalene and 0.115% of tar (reckoning on the dry coal). 75

It is an advantage of this invention that the briquetting of the agglomerate can be done without any special step of eliminating moisture; indeed, in the case of flotation concentrates, the complete treatment of the float to produce the finished briquette does not involve any drying operation. 80

What we claim as our invention and desire to secure as Letters Patent is:—

1. A process for the treatment of finely divided coal wherein the coal is suspended in water, mixed with a binding medium and subjected to heat and to agitation without aeration to ensure the agglomeration of the coal particles. 85

2. A process for the treatment of finely divided coal wherein the coal is suspended in water, mixed with a binding medium and subjected to heat and to a rolling form of agitation to eliminate air and to ensure the agglomeration of the coal particles. 90

3. A process for the treatment of finely divided coal in which the coal, suspended in water, is mixed with a binding medium in such manner as to disseminate the binding medium throughout the suspension, and the suspension is heated substantially to boiling point and subjected to a rolling form of agitation without aeration to ensure the agglomeration of the coal particles. 100

4. A process of making coal briquettes from finely divided coal in which the coal, suspended in water, is mixed with a binding medium in such manner as to disseminate the binding medium throughout the suspension and the suspension is heated substantially to boiling point and subjected to a rolling form of agitation without aeration to ensure the agglomeration of the coal particles and the agglomerates are then formed into briquettes. 110

5. A process for the treatment of finely divided coal wherein the coal is suspended in water, a binding medium is disseminated throughout the suspension by means of agitation accompanied by aeration, and the suspension is subsequently subjected to heat and to agitation without aeration to ensure the agglomeration of the coal particles. 120

6. A process of making coal briquettes from finely divided coal wherein the coal is suspended in water, a binding medium is disseminated throughout the suspension by means of agitation accompanied by aeration, and the suspension is subsequently sub- 125

jected to heat and to agitation without aeration, to ensure the agglomeration of the coal particles, and the agglomerates are then formed into briquettes.

5 7. A process for the treatment of finely divided coal wherein the coal is suspended in water and mixed with pitch and subjected to heat and to agitation without aeration to ensure the agglomeration of the coal particles.

10 8. A process for the treatment of finely divided coal wherein the coal is suspended in water and mixed with pitch together with an agent which causes the pitch when softened to spread over the surfaces of the coal particles and subjected to heat and to agitation without aeration to ensure the agglomeration of the coal particles.

15 9. A process for the treatment of finely divided coal wherein the coal is suspended in water and mixed with pitch together with naphthalene and subjected to heat and to agitation without aeration to ensure the agglomeration of the coal particles.

20 10. A process for the treatment of finely divided coal wherein the coal is suspended in water and mixed with finely divided pitch and subjected to heat and to agitation without aeration to ensure the agglomeration of the coal particles.

25 11. A process of making coal briquettes from finely divided coal in which the coal is suspended in water, is mixed with a binding medium as herein described by agitation accompanied by aeration and then the suspension is heated substantially to boiling point and subjected to a rolling form of agitation without aeration to ensure the agglomeration of the coal particles and then the agglomerates are formed into briquettes.

30 12. A process for the treatment of finely divided coal wherein the coal is suspended in water to form a mobile pulp and mixed with a binding medium and subjected to heat and to agitation without aeration to en-

sure the agglomeration of the coal particles.

35 13. The process of making coal briquettes from finely divided coal wherein the coal, suspended in water to form a mobile pulp, is mixed with a binding medium as herein described by agitation accompanied by aeration and is subsequently heated in a drum rotating on a substantially horizontal axis to ensure agglomeration of the coal particles which are then formed into briquettes.

40 14. The process of making coal briquettes from finely divided coal wherein the coal, suspended in water to form a mobile pulp, is mixed with a binding medium of the kind described by agitation accompanied by aeration and is subsequently heated in a drum rotating on a substantially horizontal axis with rolling solid bodies therein to ensure agglomeration of the coal particles which are then formed into briquettes.

45 15. The process of making coal briquettes which consists in agitating a coal pulp with a binder under such conditions that the binder will flow and coat the coal particles and further subjecting the pulp containing the coated coal particles to agitation without aeration to produce agglomerates of the coated coal particles substantially free from air, and then forming the agglomerates into briquettes.

50 16. The process of making coal briquettes which consists in agitating a heated coal pulp with a binder so that the binder will coat the coal particles, and further subjecting the pulp containing the coated coal particles to agitation without aeration to produce agglomerates of the coated coal particles substantially free from air, and then forming the agglomerates into briquettes.

55 In testimony whereof we have signed our names to this specification.

WILLIAM WARWICK STENNING.  
WALTER HENRY BEASLEY.